

S. B. HENNING.

PROCESS OF MANUFACTURING PLYWOOD.

APPLICATION FILED JUNE 19, 1918.

1,329,402.

Patented Feb. 3, 1920.

Fig. 1.



Fig. 2.



cold temperature,  
50° - 100°  
pressure

Fig. 3.



hot temperature  
50° - 100°  
pressure

Inventor:

Sherburne B. Henning  
By Robert S. Young,  
Attorney

# UNITED STATES PATENT OFFICE.

SHERBURNE B. HENNING, OF MADISON, WISCONSIN, ASSIGNOR TO THE UNITED STATES OF AMERICA.

## PROCESS OF MANUFACTURING PLYWOOD.

1,329,402.

Specification of Letters Patent.

Patented Feb. 3, 1920.

Application filed June 19, 1918. Serial No. 240,842.

To all whom it may concern:

Be it known that I, SHERBURNE B. HENNING, a citizen of United States, residing at Madison, in the county of Dane and State of Wisconsin, have invented a new and useful Improvement in Processes of Manufacturing Plywood, of which the following is a specification.

My invention relates to the manufacture 10 of waterproof plywood and consists in combining certain materials in definite proportion and then in using in a particular manner the composition prepared.

The object of my invention is the production 15 of a waterproof plywood. Plywood made in accordance with my invention is especially adapted for use as a covering for a surface which is subjected to extreme changes in moisture conditions. It may also 20 be used where a material is required which must be light and strong and will not be affected by moisture.

In the accompanying drawing:

Figure 1 illustrates three plies of material 25 to which glue may be applied;

Fig. 2 shows three plies of material in a press in which heat is not used;

Fig. 3 shows three plies of material in a press in which heat is applied in the usual 30 way.

In carrying out my invention I prepare the glue of the following ingredients using approximately the following proportions of said ingredients: one hundred (100) parts 35 by weight of powdered casein, four hundred (400) to six hundred (600) parts of water, fifteen (15) to eight (8) parts water slaked lime, and ten (10) to thirty (30) parts of dry granulated blood albumin 40 (black soluble). The albumin should be of sufficient fineness to pass through a ten (10) mesh sieve.

The casein is soaked one hour in all the water. The dry powdered lime is then added, and the mixture is stirred for about ten 45 minutes. The granulated dry blood albumin is then added to the mixture by stirring. After this mixture has stood for 15 minutes, it is ready for use.

It will be noted that the proportion of lime used varies inversely to the proportion 50 of water and blood albumin used.

In manufacturing plywood this glue is spread on the plies in any of the usual ways.

The plies are then cold pressed for about 55

one-half hour, the pressure maintained being between fifty (50) and one hundred (100) pounds per square inch. The plies are then subjected to approximately the same pressure in a hot press, the temperature of which is approximately 212° Fahrenheit. Thin plies are kept in the hot press for about two minutes while a longer period is required for thicker plies.

What I claim is:—

1. The process of manufacturing plywood, which comprises assembling a plurality of plies of fibrous material with a casein-blood adhesive between the adjacent faces thereof, subjecting the same to a relatively high cold pressure for a short period, and thereafter subjecting the same to a substantially equal hot pressure for a shorter period.

2. The process of manufacturing plywood, which comprises assembling a plurality of plies of fibrous material with a casein glue between the adjacent faces thereof, subjecting the same to a relatively high cold pressure for a short period, and thereafter subjecting the same to a substantially equal hot pressure for a shorter period.

3. The process of manufacturing plywood, which comprises assembling a plurality of plies of fibrous material with a casein-blood adhesive material between the adjacent faces thereof, subjecting the same to a cold pressure of from fifty to one hundred pounds for approximately a half hour, and thereafter subjecting the same to a substantially equal hot pressure for a shorter period.

4. The process of manufacturing plywood, which comprises assembling a plurality of plies of fibrous material with a casein glue between the adjacent faces thereof, subjecting the same to a cold pressure of from fifty to one hundred pounds for approximately a half hour, and then subjecting the same to a substantially equal hot pressure for a shorter period.

5. The process of manufacturing plywood, which comprises assembling a plurality of plies of fibrous material with an adhesive consisting of casein, water, lime, and albumin, between the adjacent faces thereof, subjecting the same to a relatively high cold pressure for a short period, and thereafter subjecting the same to a substantially equal hot pressure for a shorter period.

6. The process of manufacturing plywood,

which comprises assembling a plurality of plies of fibrous material with an adhesive comprising approximately: 100 parts by weight of powdered casein, 400 to 600 parts of water, 15 to 8 parts of water slaked lime, and 10 to 30 parts of blood albumin placed between the adjacent faces thereof, subject-

ing the same to a relatively high cold pressure for a short period, and thereafter subjecting the same to a substantially equal 10 hot pressure for a shorter period.

In testimony whereof I have hereunto affixed my signature.

SHERBURNE B. HENNING.